

Oct. 30, 1934.

J. A. MUIR

1,978,549

SHOE MATERIAL

Filed Feb. 26, 1932

Fig. 1.



Fig. 2.



Fig. 3.



Fig. 4.



Fig. 5.



Fig. 6.



Inventor

James A. Muir.

By: Lippmann, elegant, Darby & Luskman  
Attorneys

## UNITED STATES PATENT OFFICE

1,978,549

## SHOE MATERIAL

James A. Muir, Baltimore, Md., assignor to Crown Cork & Seal Company, Inc., Baltimore, Md., a corporation of New York

Application February 26, 1932, Serial No. 595,373

12 Claims. (Cl. 154—2)

The present invention relates to a new and improved sueded article and method of making the same.

An important feature of the invention is to provide a cork product composed of sheet cork or cork composition, to the surface of which, is applied by an adhesive coating, short textile fibers or other flocculent material such as wool or cotton flock, to form a durable shoe material product having a smooth sueded surface of attractive appearance and which is especially suited for use as an insole for shoes, slippers and the like.

Heretofore, in the use of cork insoles of this character, it has been necessary, due to the rough surface texture of the material, to employ a separate covering strip so as to provide a smooth and comfortable surface for the foot. The sueded cork product formed by the present invention is admirably suited for use as an insole, since it has an exposed smooth surface that is devoid of the undesirable rough texture of the sheet cork or cork composition, yet retains all its desirable properties. Moreover, as the cork product thus formed very closely resembles sueded leather it may be economically substituted therefor in the manufacture of various articles such as the uppers of shoes, slippers and the like.

A further object is to provide an article of sueded material in which the short textile fibers or flock are connected to the cork sheet or cork composition by a rubber compound, such as light elastic gum cement, to provide an exceptionally durable and rugged wearing surface.

Other objects and advantages of the invention will become apparent from the following description when taken in conjunction with the following claims and drawing.

Referring to the drawing in which is illustrated several preferred embodiments of the invention:

40 Figure 1 is a perspective view of an insole made in accordance with the invention;

Figure 2 is a sectional view taken substantially along the line 2—2 of Figure 1;

Figure 3 is a perspective view of a modified form of the invention;

Figure 4 is a sectional view taken substantially along the line 4—4 of Figure 3;

Figure 5 is a sectional view of a further modification; and

50 Figure 6 is a sectional view of another form of the invention.

Referring to the drawing in which like numerals indicate like parts in the several views, 10 denotes a cork insole for shoes, slippers or the like, 55 which is preferably composed of a base 11 of sheet

cork or cork composition formed of comminuted or ground cork, which, after being thoroughly mixed with a binder, is passed through a calendar to form a flexible and compact sheet. The upper surface of the cork base 11 is then coated with adhesive material 12 on which is sprinkled or blown minute textile fibers or other flocculent material 13 such as flocks of wool or cotton to provide an exposed sueded surface.

As an alternative procedure the flock may be applied to the cork composition sheet while the binder of the sheet is soft, thereby constituting the binder as the adhesive for uniting the flock to the sheet and making unnecessary the later application of an adhesive coating. It will be understood, therefore, that in this procedure, as well as in the previously described method, I provide a cork composition sheet having an adhesive surface and apply flocculent material to such surface.

While any suitable adhesive may be employed, it has been found that an efficient binder is obtained by mixing oxidized linseed oil or other allied oils together with kauri gum and rosin. Also a binder of the varnish type in which pyroxylin and varnish oils are incorporated with a suitable drier may be used. The surplus flock is then removed by a vacuum or the like and the material may be passed through a suitable drier to properly cure the adhesive.

The shoe material formed, provides a product which, on one side, has the natural color of cork, and on the other side the appearance of sueded leather or mole-skin and because of its relative lightness, flexibility, resiliency, insulating, cushioning, and ventilating properties, may be applied to various uses. The combination of the cork and suede impart to the insole the desired resiliency and smoothness and also acts as a shock absorber to produce the same cushion effect as rubber, but which eliminates rubber completely from the composition, since the latter has a tendency, when used in an insole, to draw in the foot and make the shoe feel uncomfortable.

The cork composition or a substitute thereof (Fig. 3) may also have applied to its upper surface in its formative stage, a backing or carrier strip of reinforced fabric 15 which is embedded or keyed to the cork composition 14 in any suitable manner. To the fabric 15 is applied the adhesive 16 and the flocculent material 17 to provide a smooth exposed sueded surface.

As shown in Figure 5, the cork composition 18 has applied to both sides thereof an adhesive 19 on which is sprinkled the short fibers or flocculent

material 20 to form a product having opposed sueded surfaces.

By the shoe material as referred to, is included upper material, insoles, box toes, counters, and other parts used in the construction of boots, shoes, and slippers.

Where it is desired to provide an especially durable sueded surface, instead of employing the adhesive cement binder, there may be substituted therefor, as shown in Figure 6, a rubber compound 21 such as elastic gum mixed with a latex composition. The rubber compound is first applied to the cork sheet or cork composition 22 to constitute a fill or anchor coat on the cork. Immediately, a second coat of elastic gum 23 containing therein fine particles of flocculent material, textile fibers or their equivalent is compressed into the cork surface 22. While the surface of the elastic gum containing the flocculent material 20 is still sticky, additional dry flock 24 is spread under pressure on the adhesive surface thus formed. The surplus remaining flock is removed in any suitable manner, such as by suction or the like. The sheet material is then vulcanized, 25 which results in the finished, smooth, sueded product, that is especially adapted for use, where strength and durability without increased weight are desired, additionally, the sueded cork product, due to its waterproof properties, render it 30 suitable as an economical substitute for rubber products such as raincoats and the like, yet is entirely free of the undesirable tendency of rubber to retain and condense moisture.

It is to be understood that the forms of the invention shown and described are merely illustrative of preferred embodiments and such changes may be made as fall within the purview of one skilled in the art and the scope of the appended claims.

40 What I claim is:

1. A new and improved process of forming sueded material which consists in applying to a cork composition sheet gum cement, then applying a second coat of gum cement containing fine 45 particles of flock or textile fibers, and while the surface of cement containing the flock is sticky applying dry flock thereto.

2. A new and improved process of forming sueded material which consists in applying to a cork composition sheet gum cement, then applying a second coat of gum cement containing fine 55 particles of flock or textile fibers, while the surface of cement containing the flock is sticky applying dry flock thereto, and vulcanizing the layers thus formed to provide a sueded surface.

3. As a new article of manufacture, an insole comprising a flexible and compact base formed of a mixture of comminuted cork and a binder, said base having a coating of flocculent material adhesively united thereto so as to form a sueded surface.

4. As a new article of manufacture, an insole including a calendered base of comminuted cork

and a binder mixture having a textile reinforcing layer united thereto and a coating of flocculent material adhesively united to the base to provide a smooth sueded surface.

5. As a new article of manufacture, an insole strip including a calendered base of comminuted cork and a binder mixture having a textile reinforcing layer united thereto and a coating of flocculent material adhesively united to the reinforcing layer to provide a smooth sueded surface. 80

6. As a new article of manufacture an insole comprising a flexible and compact base formed of a mixture of comminuted cork and a binder, said base having a coating of flocculent material adhesively united to each side thereof to provide 85 outer sueded surfaces.

7. As a new article of manufacture, an insole comprising a flexible and compact base formed of a mixture of comminuted cork and a binder, said base having a coating containing particles 90 of flocculent material mixed throughout the body of the coating, and dry flock adhesively united to the coating to form a sueded surface.

8. The method of producing an insole which consists in forming a flexible and compact base 100 from a mixture of comminuted cork and a binder, coating the base with an adhesive and applying to the adhesive coating before it hardens a flocculent material, thereafter permitting the adhesive to harden and form a smooth sueded surface. 105

9. A new and improved process of forming sueded shoe material which consists in forming a base of comminuted cork, the particles of which are adhesively connected by a binder, calendering 110 the base to form a flexible and compact sheet, coating the base with adhesive and applying flocculent material to the adhesive.

10. A new and improved process of forming sueded shoe material which consists in forming a 115 base of comminuted cork, the particles of which are adhesively united by a binder, calendering the base to form a flexible and compact sheet, coating the sheet with vulcanizable adhesive, applying flocculent material to the adhesive and vulcanizing the layers thus formed to provide a sueded surface. 120

11. A new and improved process of forming sueded shoe material which consists in forming a base of comminuted cork, the particles of which 125 are adhesively united by a binder, calendering the base to form a flexible and compact sheet, coating the sheet with adhesive having flocculent material mixed in the body thereof, applying dry flocculent material to the coated surface, compressing 130 the layers thus formed, removing the surplus fibers and subjecting the material to a drying operation.

12. An insole having a base of comminuted cork and a suede-like surface affixed to one side of the 135 base.

JAMES A. MUIR.